

**United States Patent [19]**  
**McCready**

**[11] Patent Number:** 4,647,353  
**[45] Date of Patent:** Mar. 3, 1987

**[54] CATHODIC PROTECTION SYSTEM**

**[76] Inventor:** David McCready, P.O. Box 1971, Altoona, Pa. 16603

**[21] Appl. No.:** 817,656

**[22] Filed:** Jan. 10, 1986

**[51] Int. Cl.:** C23F 13/00

**[52] U.S. Cl.:** 204/147; 204/196; 204/294; 106/74; 106/84; 106/287.23; 106/287.29; 106/287.35

**[58] Field of Search:** 204/147, 148, 196, 197, 204/286, 297 R, 294

**[56] References Cited**

**U.S. PATENT DOCUMENTS**

|           |        |               |         |
|-----------|--------|---------------|---------|
| 2,776,940 | 1/1957 | Oliver        | 204/196 |
| 2,870,074 | 1/1959 | Parker        | 204/294 |
| 3,151,050 | 9/1964 | Wilburn       | 204/196 |
| 3,377,150 | 4/1968 | Corley et al. | 204/294 |

|           |         |                 |           |
|-----------|---------|-----------------|-----------|
| 3,410,772 | 11/1968 | Geld et al.     | 204/196   |
| 3,498,898 | 3/1970  | Bogart et al.   | 204/196   |
| 3,632,444 | 1/1972  | Grotheer et al. | 204/294   |
| 3,868,313 | 2/1975  | Gay             | 204/196   |
| 3,893,903 | 7/1975  | Lindholm        | 204/197   |
| 3,933,613 | 1/1976  | Turner          | 204/297 R |
| 4,226,694 | 10/1980 | Babolian et al. | 204/196   |

**FOREIGN PATENT DOCUMENTS**

1227405 4/1971 United Kingdom 204/294

*Primary Examiner—T. Tung*  
*Attorney, Agent, or Firm—James C. Wray*

**[57]**

**ABSTRACT**

An anode of about 98% carbon, 2% silica gel and less than 1% inert binders is mounted on a layer spread on a metal surface.

17 Claims, 2 Drawing Figures





## CATHODIC PROTECTION SYSTEM

## BACKGROUND OF THE INVENTION

The invention relates to automotive cathodic protection devices and more in particular to the structure of the anodes used to impress a current within the automotive body.

Automobiles of all types must be able to cope with varying degrees of inclement weather. When moisture increases, protective measures against automobile body corrosion should be intensified. Extant carbon anodes which are used in cathodic protective systems are deficient in the ability to respond to varying degrees of moisture. What is needed in the art is a carbon anode which can respond to varying degrees of atmospheric moisture so that as humidity increases conductivity to protected surfaces also increases.

## SUMMARY OF THE INVENTION

The invention is essentially a composite carbon anode for use in automotive cathodic protection devices with means for attaching it to a car body and effecting good electrical conductivity therewith. The composite material is deemed carbosil which reflects the carbon and silica gel components.

One of the most salient features of the invention is the anode's ability to respond to variations in humidity. It should be appreciated that as humidity increases protection against corrosive forces should also increase. The invention provides an anode which is responsive to variations in humidity such that as humidity increases the electrical conductivity between the anode and the car surface also increases.

A preferred embodiment for an anode apparatus for use in automotive cathodic protection devices comprises a layer of anode enhancement liquid spread upon a bare metal surface. This bare metal surface should have a hole extending therethrough for receiving a fastener. The substantially carbon anode then is 40 mounted on this layer. The anode also has a hole extending therethrough which is to be aligned with the hole on the surface. An electrical lead is then attached to the anode by way of a ring connector. The ring is held in alignment with the holes through which a plastic 45 threaded fastener is inserted and secured on another side of the surface with a plastic nut. The plastic threaded fastener and nut are preferred to be made of plastic such as a nylon or polyamide. This is so that if overtightening occurs the nut will strip before the 50 anode is crushed.

The preferred anode is composed of sintered materials wherein about 90-99% of the material is carbon and preferably 98% is carbon. About 1-9% is silica gel and preferably 2% is silica gel. About 0.1-1% is inert binders and preferably less than 1% is inert binders.

The automotive enhancement liquid comprises about 41%  $H_2O$ , about 24% polyvinyl acetate-acrylic resin, about 23% calcium silicate pigment, about 4% sodium silicate stabilizer, about 3% of a 10% solution of  $H_2PO_3$ , about 3% of a 10% solution of tannic acid, about 1.5% glycol esters and about 0.5% inert material.

The preferred anode is about 5/16 of an inch thick.

The method for attaching the inventive anode to the car body for use with automotive cathodic protection devices comprises relatively few steps. One merely bares a patch of metal surface and spreads a layer of the anode enhancement liquid over this bare metal surface.

A hole is made on said surface which extends through the surface for attaching purposes. The carbon anode is then placed on this layer. An electrical lead having a ring connector is then attached to the exposed surface of the anode by way of a plastic threaded fastener inserted through the ring connector, the anode and the surface. The threaded fastener is held fast by way of a plastic nut.

It is an object of this invention to improve automotive cathodic protection devices by providing novel anode compositions.

It is another object of this invention to provide an anode responsive to variations in humidity.

It is another object of this invention to provide an anode which increases electrical conductivity with metal surfaces in response to increases in humidity.

It is another object of this invention to increase the longevity of automobile bodies.

These and other and further objects and features of the invention are apparent in the disclosure which includes the above and below specification and claims and drawings.

## BRIEF DESCRIPTION OF THE DRAWINGS

FIG. 1 is an elevated exploded perspective of the invention.

FIG. 2 is an elevated perspective of a prepared surface which would receive the embodiment of FIG. 1.

## DESCRIPTION OF THE PREFERRED EMBODIMENT

The preferred embodiment is a carbon anode with accompanying means for attachment to be used with automotive cathodic protection devices. The preferred embodiment is of the impressed-current protection device type.

When iron and other metals are placed in contact with electrolytes (water and dissolved salts from road de-icers, industrial pollution, etc.), they take on a force that desires release. This force causes the metal to dissolve into the surrounding electrolyte, after which the metals usually combine with oxygen to form oxides (rust corrosion). This is simply the action of metals returning to their most natural state.

Corrosion is a continuous electrical chemical process resulting in the destruction of metals. This corrosion is a direct result of an electrical current caused by the reaction between metal surfaces and existing chemicals found on and about vehicles. These chemicals, referred to as salts, form when substances in the road de-icing agents and industrial air pollutants combine with the atmosphere to produce active electrolytes such as  $H_2SO_4$  (common battery acid),  $HCl$ ,  $HNO_3$  and a wide spectrum of additional electrolyte-producing chemicals. Sea spray along coastal areas is another source of destructive electrolyte-producing salts, and corrosion-inducing substances can even be present in the tap water used to wash and preserve a car's finish.

The metal components of cars produce an electrical current when differences in electrical potential exist. These differences in potential are an inherent characteristic of dissimilar metal used in automobile construction. When an electrolyte is present, a path of electrons (electric current) will be released when the electrolyte contacts alloys and bolted or welded areas of the vehicle. The effect of current flow from one portion of the metal through the electrolyte to another part of the

structure causes metal ions or particles to leave the surface of the metal. As these particles separate from the structure, combining with the electrolyte, pits develop. These pits act as miniature galvanic (battery) cells. As this electrical chemical process continues, the cells grow larger and larger with the end result being the ultimate destruction of the metal. The rate of this naturally occurring current flow determines the life of the metal. For instance, one ampere of current discharge from iron is sufficient to remove 20.2 pounds of metal in a single year.

With steel, rust is solid evidence of corrosion. Rust has the same chemical composition as hematite, the most common form of iron ore. Steel mills use large amounts of energy to drive off oxygen in converting ore to steel. The reverse process is fairly passive because steel is eager to reunite with oxygen and revert back to its original state as an oxide of iron.

For metal to corrode there must be an anode, a cathode, and an electrolyte with available oxygen (usually damp earth or water). There must also be a potential difference between the anode and the cathode. These conditions set up what is called the "corrosion cell." At the anode, positively charged atoms of the metal leave the solid surface and enter the electrolyte as metallic ions. Current leaves the metal at the anode and migrates through the electrolyte to the cathode. Heat, such as is provided by sunlight, makes the reaction more efficient. This results in rust, pitting, and corrosion at the anode.

Once corrosion starts it is self-sustaining and irreversible. Age and condition of structure, coating, temperature, and other facts influence the rate of corrosion. If not controlled, corrosion, rust and pitting will continue until the metal structure is useless.

A scratch or nick in the protective coating sets the stage for rust and corrosion. When base steel is exposed to the electrolyte, the electro-chemical circuit is established. The steel gives up metallic ions to the electrolyte. A pit forms. Rust is created. The cycle is self-sustaining and will continue until the steel is consumed. Rust is formed by the uniting of the oxygen in the water and metallic ions. Many times this out-of-sight, out-of-mind process goes undetected until severe damage occurs.

A second form of corrosion, called "galvanic corrosion" happens when two dissimilar metals are in contact in the presence of an electrolyte. The metal with the higher potential becomes the anode and the one with the lower potential, the cathode. Such corrosion "cells" rob the higher-potential metal of ions until it is consumed. Metals are listed according to potential in the electromotive, galvanic, series of metals.

From the active end to the noble or passive end there is: magnesium, aluminum, iron (ferrous), cadmium, nickel, tin, brass, copper, silver, monel, titanium, platinum, graphite, gold.

Any metal higher on the scale sacrifices itself to any metal lower on the scale when the two are in contact in the presence of an electrolyte. Such sacrifice corrosion is the basis for cathodic protection.

The very nature of galvanic corrosion offers an opportunity to use it creatively. This is done by placing expendable and replaceable metal anodes (higher in the galvanic series than steel) in contact with the submerged steel to be protected. The anodes make the entire wetted steel surface a cathode and sacrifice themselves to protect the steel. Thus corrosion is used to fight corrosion.

Another means of controlling corrosion is to reverse the corrosion cell's current flow via an impressed current. Direct current is applied to an anode made of platinum, graphite, cast iron, aluminum or other material based on economic factors. The direct current reverses the galvanic flow from the steel and converts the steel into the protected cathode.

The cathodic device reduces automotive corrosion and rust by using integrated circuitry to impress a DC current on and about the car's body and support structure. This DC current, supplied by the car's battery, impedes the process by which road salts, industrial pollutants, salt air, and acid rain eat away and destroy metal components.

The system comprising the preferred embodiment consists of a command module mounted near the vehicle operator, an interface module located under the dash, and two special electrodes mounted on the front and rear of the car's underbody.

This device fights automotive corrosion where it starts by protecting concealed underbody and frame panels as well as painted outerbody surfaces that have been chipped or scratched. The very principle from which the automotive cathodic protection systems was designed ensures that the device's electrical counteraction will work hardest on those areas most susceptible to rust and corrosion. State of the art integrated circuitry and silicon chips monitor and respond to subtle changes in humidity, temperature, and other variables affecting rust formation, so the system offers maximum protection in all types of conditions. The system is compatible with sophisticated spray-on protective materials, none of which have proven lastingly effective against corrosion. The system can be considered a backup to any other rust-proofing method.

While no anticorrosion method can claim to be 100% effective the system when used as directed, can extend the life of a car's body by 75%. This means that the average car body life of eight years could be extended to 14 years. The dollar savings are obvious as evidenced by the potential for a much greater resale value beyond the fourth year of an automobile's life.

The only way to satisfy the electromotive forces set up by the electrolyte is to supply a readily available source of charged particles to act as current. Unfortunately, in vehicles unprotected by the system, the source of charged particles must be the metal itself, and rust and corrosion result.

The system supplies current to the electrolytes so a car's metals do not have to. Through the use of a car's battery and two strategically placed anodes, the device converts an entire car into a functioning cathode that supplies an electron flow to the entire car surface. Therefore, when a naturally occurring electrolyte creates a potential difference between metal parts of a car, the source for current flow becomes the car's battery, not its metal components. The effects of the electrolyte are disarmed by this superficial current flow, and the metal remains intact. Once the electrolyte is disarmed in this manner, rust and corrosion are drastically diminished.

Surface rust is very common in the dry and arid regions of the Southwest where the lack of rainfall and humidity prevents the formation of electrolytes. It is not uncommon to find 20 to 30 year old vehicles, mechanically worn out and abandoned, having solid bodies almost completely devoid of paint. These vehicles do not rot away with cavernous holes. Complete destruc-

tion of body panels and frame members simply does not occur because corrosion cannot begin without the presence of an electrolyte.

These vehicles have one extremely interesting point in common, i.e., their entire surface may have a red dust coating of iron oxide. This is because areas of extremely low humidity, oxygen in the atmosphere combines with iron to produce ferric oxide hydrate, a crystalline compound that acts as a barrier against further oxidation of the iron. If an electrolyte were present, deep penetrating corrosion could occur, but because of the extreme lack of moisture, oxidation ceases almost immediately. For these reasons, it is completely normal to see this extremely light coating of surface rust even when using the system.

Aside from erosion by sand and small stones abrading away body panels, all automotive corrosion is the result of the electro-chemical reaction set off by electrolytes. Poltice corrosion is a severe form of corrosion most often found in the underbody fender wells where mud, road salt, and moisture collect, forming a poltice. The salt in this poltice draws even more moisture from the atmosphere, making these areas prone to continuous corrosion action.

Stress corrosion occurs as a result of torsional effect on metal components. This torsional effect can be caused in one of two ways: (a) by the normal stress and movement of metal resulting from normal movement and vibration; or (b) by impact bending of body panels caused by external forces such as slight collisions with pebbles, other cars, or other objects. As the metal flexes, its crystalline structure gives way and releases metal ions.

Starting with a difference in potential, rust and corrosion is always the result.

Potential Difference. A potential difference is unavoidably built into steel during its manufacture. When steel is exposed to an electrolyte and oxygen, an electrochemical reaction takes place.

Temperature variations, such as sunlight on one side of a tank, can set up strong potential differences. Or, a combination of agitated and stagnant water areas is a condition that encourages corrosion.

Welds corrode fast. Heat from welding changes the potential in the weld area (charged particles of metal). These metal ions then react with the electrolyte, speeding up the corrosion process in the affected area.

Pit corrosion (described earlier) can occur whenever favorable conditions exist. But it is interesting to note that it is most active during a wetting/drying cycle, when the corrosion rate is actually enhanced and the pitting attack is most rapid. This pitting is not limited to cold weather. In fact, pitting activity increases as the temperature increases.

The real demons of rust and corrosion are electrolytes that permit electrical activity between the dissimilar metals and alloys of a car's frame and body components. The system provides the necessary electrons to disarm and render these electrolytes less active.

For corrosion in a joint a potential difference is set up between the oxygen-rich electrolyte and oxygen-starved electrolyte at the bottom of the crevice. This condition can occur at joints and welds where water is stagnant.

Pressure or stress in one area can change potential. Most times, the point of stress becomes an anode. This weakens the steel where strength is most needed. Stress

points, such as bends or surface hardened areas, are good candidates for corrosion.

In the past 25 years the most common method of "rust proofing" car bodies involved spraying them with protective undercoatings. While these coatings do provide a certain amount of sound absorption and abrasion resistance, their record as corrosion inhibitors has proven less than effective. Application is difficult, and many corrosion-vulnerable areas of a car cannot be reached by even the most sophisticated spraying equipment. Furthermore, in as little as two and a half to four years, coated vehicles have shown extensive corrosion beneath the protective coating. This is because no matter how good the protective coating, electrolytes can eventually work their way through the coating to the metal below by the process of osmosis. This is why the device can serve as an effective backup to even the most respected undercoating systems.

Electrolytes can penetrate protective coatings by osmosis and attack the metal beneath. The coating will actually flake off the metal.

A car's battery is an ideal source of energy to power a cathodic protection device since it supplies direct current, the exact type of electrical current needed for this type of protection. Of course, the device does draw a small amount of power from the battery at all times, but when compared to the savings on the car's body, the wear on the battery is truly negligible. For example, under normal use (driving a car 100 or more miles per week), the battery will have sufficient opportunity to recharge. If a car is stored for 30 days without operating it, there will be an appreciable drain on the battery, but most good quality batteries will still retain enough reserve to start the engine and begin the recharging cycle. The device also incorporates a unique pulsating system that allows a battery to use its rejuvenating properties more effectively.

Cathodic protection is not new. It has been used extensively to protect underground pipelines, reinforcement bars on bridges, and ocean going vessels. Industries with high capital investment, such as petroleum, shipping, construction, and exploration, have always recognized the value of extending the useful life of their metal goods.

In the automobile industry, the incentive to extend the life of the product simply did not exist.

Reasoning that it would cut down future sales, those in the industry considered it unthinkable to build a vehicle that would last beyond ten years.

In accordance with the device described above, the invention provides carbon anodes. The composition of the anodes is about 98% carbon and about 2% silica gel, with less than 1% of the anode containing inert binders.

55 The components are sintered, then combined homogeneously, evenly mixed, and extruded as a high density compressed mass. The material is reduced to specific anode size as required. This anode is deemed Carbosil to reflect the carbon and silica nature of the composite.

60 The Carbosil anode has been designed to meet requirements of impressed current design. The dessicants, i.e., less than 5% of total composition, are sensitive to atmospheric moisture and thereby vary conductivity to protective surfaces. As the humidity increases, the associated electrolytic corrosion effect increases. In response,

65 the carbosil anode increases the conductivity to protective surfaces. Therefore, the addition of moisture-sensitive compounds to the carbon anodes increases the

distribution of current necessary to disarm the corrosive effect of the electrolyte.

The properties of the Carbosil anode are:

- a. Bulk Density—0.0625 lbs/cu. in.
- b. Maximum Grain Size—0.035 inch
- c. Specific Resistance—0.00039 ohms/in.
- d. Compression Strength—5200 PSI
- e. Porosity—25%
- f. Tensile Strength—1800 PSI
- g. Thermal Conductivity—0.25 BTU/FT<sup>2</sup>sec.F.

Referring now to FIG. 1, the anode with attaching means will be discussed with particularity. There is the anode itself 16. The sintered material is generally indicated by the numeral 10. The side of the anode to be in contact with the car body is 14. The side of the anode to which the electrical lead attaches is 12. The threaded fastener for attaching the anode 16 to the car body is 40. It is preferred this be of a plastic or a dielectric material such as a polyamide, i.e., nylon. The electrical lead 32 has a ring connector 30 attached to the electrical lead. The ring connector has a sleeve 34 adapted to receive the lead 32. The ring 36 has a hole 38 through which threaded fastener 40 may be inserted. The hole 38 is in alignment with hole 18.

FIG. 2 depicts a section of car body. A hole 28 extends therethrough for receiving threaded fastener 40. The area encompassed by dotted line 22 represents the bare metal surface which has had paint removed from it. This surface, 24, would be the primary area of conductance. The area encompassed by line 26 is the area 30 which has been coated with the anode enhancement liquid. Essentially, a surface of the metal has been cleaned free of any coating material and then has been painted, with a little bit of overlap onto coated areas, with an enhancement or electrical enhancement material. This material comprises: 41% H<sub>2</sub>O, 24% polyvinyl acetate-acrylic resin, 23% calcium silicate pigment, 4% sodium silicate stabilizer, 3% of a 10% molar solution of phosphoric acid, 3% of a 10% molar solution of tannic acid, 1.5% glycol esters and 0.5% inert material. The 40 purpose of the fluid is to enhance the electrical conductivity of the surface 24.

The surface 20 on FIG. 2 is that area of the car body surface which has not been touched with the process of attaching the invention.

On a back side of surface 24 there is located a plastic dielectric nut 25 for receiving the threaded fastener 40. It is important that this nut be made of a polyamide or similar material such that when overtightening occurs the nut will strip before the anode is crushed.

As this invention may be embodied in several forms without departing from the spirit or essential characteristics thereof, the present embodiment is therefore illustrative and not restrictive, and whereas the scope of the invention is defined by the appended claims, all changes that fall within the metes and bounds of the claims or that their form their functional as well as their conjointly cooperative equivalents are therefore intended to be embraced by those claims.

What I claim is:

1. An anode apparatus for automotive cathodic protection devices, comprising:

- (a) a layer spread upon a bare metal surface wherein said surface has a hole extending therethrough for receiving a fastener;
- (b) a substantially carbon anode mounted on said layer and having a hole extending therethrough for receiving a fastener, said anode being composed of

sintered material and, comprising about 90-99% carbon about 1-9% silica gel, and about 0.1-1% inert binders

- 5 (c) an electric lead attached to said anode;
- (d) a plastic threaded fastener extending through said holes, whereby said anode with the lead is held fast to said surface.

2. The apparatus of claim 1 wherein said fastener further comprises a plastic nut for receiving said fastener in threaded engagement, said nut located on a back side of said surface.

15 3. The apparatus of claim 2 wherein said layer further comprises about 41% H<sub>2</sub>O, about 24% polyvinyl acetate-acrylic resin, about 23% calcium silicate pigment, about 4% sodium silicate stabilizer, about 3% of a 10% solution of H<sub>2</sub>PO<sub>3</sub>, about 3% of a 10% solution of tannic acid, about 1.5% glycol esters and about 0.5% inert material.

20 4. The apparatus of claim 1 wherein said anode is about 5/16ths of an inch thick.

5. The apparatus of claim 4 wherein said fastener is composed of a polyamide.

6. The apparatus of claim 5 wherein said lead has a ring connector through which said fastener is received, whereby said lead is held fast to a surface of said anode.

7. An anode apparatus for automotive cathodic protection devices, comprising:

- (a) a layer of liquid spread upon a bare metal surface, wherein said surface has a hole extending therethrough for receiving a fastener, and wherein said liquid is about 41% H<sub>2</sub>O, about 24% polyvinyl acetate-acrylic resin, about 23% calcium silicate pigment, about 4% sodium silicate stabilizer, about 3% of a 10% solution of H<sub>2</sub>PO<sub>3</sub>, about 3% of a 10% solution of tannic acid, about 1.5% glycol ester and about 0.5% inert material;
- (b) a substantially carbon anode mounted on said layer and having a hole extending therethrough for receiving a fastener, wherein said anode further comprises about 90-99% carbon, about 1-9% silica gel, and about 0.1-1% inert binders;
- (c) an electric lead attached to said anode, wherein said electric lead has a ring connector through which said fastener may be received, whereby said fastener is held fast to a surface of said anode;
- (d) a plastic threaded fastener extending through said hole, whereby said anode with the lead is held fast to said surface, said plastic fastener further comprising a plastic nut for receiving said threaded fastener in threaded engagement, said nut located on a back side of said surface, and wherein said plastic threaded fastener and nut is composed of a polyamide.

55 8. The apparatus of claim 7 wherein said anode is composed of sintered material.

9. The apparatus of claim 8 wherein said anode is about 5/16th of an inch thick.

10. A method for attaching an anode to a car body for use with an automotive cathodic protection device, comprising the steps of:

- (a) barring a patch of metal surface; and
- (b) spreading a layer of liquid over said bare metal surface; and
- (c) providing a hole through said layer and said bare metal surface;
- (d) placing on said layer, a carbon anode comprising 97-98% carbon about 1.9-2% silica gel and 0-1% inert binders.

11. The method of claim 10 wherein said anode is composed of sintered material.

12. The method of claim 11 wherein said step of spreading a layer of liquid is carried out using a liquid comprising about 41% H<sub>2</sub>O, about 24% polyvinyl acetate-acrylic resin, about 23% calcium silicate pigments, about 4% sodium silicate stabilizer, about 3% of a 10% solution of H<sub>2</sub>PO<sub>3</sub>, about 3% of a 10% solution of tannic acid, about 1.5% glycol esters and about 0.5% inert material.

13. An anode apparatus for cathodic protection devices comprising a solid material having from about 90 to about 99 percent carbon and from about 1 to about 9 percent silica gel and from about 0.1 to about 1 percent inert binder.

14. The apparatus of claim 13 wherein the components are sintered, combined homogeneously, evenly mixed and extruded as a high density compressed mass.

15. The apparatus of claim 13 wherein the carbon comprises about 98 percent, the silica gel comprises about 2 percent and the inert binder comprises about less than 1 percent of the anode.

16. The apparatus of claim 3 wherein the anode is about 5/16th of an inch thick and has a central opening extending therethrough and further comprising a connector ring, and a fastener extending through the connector ring and opening and a nut distally mounted on

10 the fastener.

17. The apparatus of claim 13 wherein the anode has a bulk density of about 0.0625 pounds per cubic inch, a minimum grain size of about 0.035 inch, a specific resistance of about 0.00039 ohms per inch, a compression strength of about 5200 psi, a porosity of about 25 percent, a tensile strength of about 1800 psi and a thermal conductivity of about 0.25 BTUs per square foot sec. f.

\* \* \* \* \*